

## UNITED STATES PATENT OFFICE

GEORGE A. RICHTER, OF BERLIN, NEW HAMPSHIRE, ASSIGNOR TO BROWN COMPANY,  
OF BERLIN, NEW HAMPSHIRE, A CORPORATION OF MAINE

## CHEMICAL PROCESSING OF CELLULOSE PULPS

No Drawing.

Application filed April 15, 1929. Serial No. 355,428.

This invention relates to the chemical processing of cellulose pulps to improve their quality, and, while not limited thereto, is more especially concerned with the chemical processing of those types of wood pulp produced by alkaline cooking processes such as the kraft or the soda process.

There are various processes of liberating cellulose fiber from raw cellulosic materials such as wood, each of which yields a pulp having more or less well-defined physical and chemical characteristics, even though similar raw cellulosic materials be used in the various processes. For instance, wood pulp produced by the acid sulphite process in which the cooking liquor consists of a sulphurous acid solution of a sulphite is distinctly different physically and chemically from wood pulp produced by the kraft process in which the cooking or kraft liquor consists of a solution of caustic soda and sodium sulphide, even though spruce chips constitute the raw cellulosic material. The differences between the various types of pulp may be ascribed to the difference in action of the cooking liquors employed upon raw cellulosic material, an acid-sulphite liquor, for instance, being more effective in its action upon ligneous matter and pentosans associated with raw cellulosic material such as wood, than alkaline liquor such as kraft liquor, with the result that sulphite pulp has a lower ligneous and pentosan content and is lighter in color than kraft pulp. Sulphite pulp may therefore be readily bleached to whiteness, whereas the bleaching of kraft pulp is accompanied by much higher bleach usage and results in a marked physical and chemical degradation of the fiber. Sulphite pulp is, however, distinctly inferior in its physical characteristics, including strength and tear resistance, to kraft pulp, doubtless as a result of the hydrolyzing action of the acid-sulphite liquor upon the cellulose fibers during the cooking operation.

The object of the present invention is to convert cellulose pulp such as kraft or soda pulp, (previously liberated by digestion of wood chips in an alkaline cooking liquor), into a white fiber of higher alpha cellulose content and yet having approximately the

physical characteristics, including strength and tear resistance, of the original kraft or soda pulp. In my application Ser. No. 40,959, filed July 1, 1925, this object is attained by digesting the kraft or soda pulp in an acid-sulphite liquor having a combined <sup>65</sup>  $\text{SO}_2$  content higher than its free  $\text{SO}_2$  content, and then bleaching the digested fiber. It is stated in that application that a sulphite liquor containing more combined than free  $\text{SO}_2$  is capable of removing a substantial proportion of impurities, especially pentosans, from pulp such as kraft, and that kraft pulp when digested in such liquor may be bleached to a whiteness of the usual bleached sulphite <sup>60</sup> pulp without being depreciated in its physical characteristics. It is further stated in that application that when digestion of such pulp is effected in an acid-sulphite liquor containing more free than combined  $\text{SO}_2$ , the resulting pulp is degraded physically and its strength and tear resistance are considerably lower than that of the original pulp. The resulting pulp is also lower in alpha cellulose <sup>65</sup> content than the original pulp and has lost other physical characteristics associated with the original pulp.

In carrying out an acid sulphite digestion of kraft pulp with a liquor containing more combined than free  $\text{SO}_2$ , it is necessary to permit a long period of contact between pulp and liquor in order to ensure the desired reaction upon and removal of impurities associated with the pulp. For instance, if such digestion is carried out at boiling temperature and under atmospheric pressure, the time required may be from six to ten hours, and even if digestion is carried out at considerably higher temperatures and under super-atmospheric pressure, the time required may be from two to four hours. On the other hand, digestion of kraft pulp in an acid-sulphite liquor containing more free than combined  $\text{SO}_2$  results in a removal of impurities in a much shorter <sup>70</sup> time. Apparently, higher free than combined  $\text{SO}_2$  content in the liquor is accompanied by a more rapid reaction upon and solution of impurities such as ligneous matter and pentosans from the fiber, the action probably being <sup>75</sup> analogous to that of a cooking liquor contain-

ing high free  $\text{SO}_2$  content upon raw cellulosic material, it being well known that a high free  $\text{SO}_2$  content in the cooking liquor is accompanied by a rapid liberation of fiber, as a result of rapid hydrolysis and solution of lignous matter, pentosans, and other cementitious material. It is also known that the higher the free  $\text{SO}_2$  content of an acid-sulphite cooking liquor, the lower the temperature and pressure required for completing fiber liberation.

As previously stated, however, an acid-sulphite liquor containing more free than combined  $\text{SO}_2$  degrades or injures a pulp markedly. For instance, assuming that one starts with kraft pulp having a pentosan content of 8% to 10%, a slowness of 10 minutes, a strength of 150, a tear resistance of 250, and a brown color, and digests such pulp at 212° F. as a 6% suspension in an acid sulphite liquor containing 2% free  $\text{SO}_2$  and 1% combined  $\text{SO}_2$  for two to three hours, the product will have a pentosan content of from 3% to 5%, a slowness of about 20 to 30 minutes, a strength of about 110 to 120, and a tear resistance of 140 to 160, and will be lighter in color. This product may be bleached to whiteness with considerably less bleach than is required for the original kraft pulp, but the bleached product has physical characteristics departing markedly from the original kraft pulp.

The present invention differs from the prior processes, thus described, in that the kraft pulp, liberated and recovered from the wood by digestion in an alkaline working liquor, is subjected first, to digestion in an acid-sulphite liquor and second, to a digestion in an alkaline liquor, as a result of which certain benefits and advantages are secured as will be set forth. I have found, for example, that if kraft pulp which has been injured by digestion in an acid-sulphite liquor, containing more free than combined  $\text{SO}_2$ , is then digested with an alkaline liquor to remove products of hydrolysis resulting from the acid-sulphite treatment, the fiber is remarkably improved in physical and chemical characteristics, its strength and tear resistance being increased to values comparable with those of the original pulp. The alpha cellulose content of the final product will be 91% to 95%, if sufficient alkali is present in the alkaline liquor. The resulting alkaline-digested pulp is readily bleachable to whiteness with a comparatively small amount of bleach, substantially without affecting its physical characteristics. The resulting final white product is accordingly an excellent raw material for the manufacture of high grade papers and for use in the preparation of cellulose derivatives.

A kraft pulp which has been digested as hereinbefore described in an acid-sulphite liquor having more free than combined  $\text{SO}_2$  may be washed and digested in alkaline

liquors of various compositions and under various temperature and pressure conditions. For example, the acid-sulphite-digested kraft pulp, after washing, may be digested as a 6% suspension in a caustic soda liquor containing from 8% to 12% NaOH, based on fiber, at 212° F. for about six hours, at the end of which time a finished product having the physical and chemical characteristics hereinbefore given is obtained. If desired, alkaline digestion may be carried out in closed digesters at higher temperatures, say at about 300° F., in which case less time is required to produce the desired product. If desired, a portion or all of the caustic soda may be replaced by alkalies such as sodium sulphide, sodium carbonate, or sodium sulphite, these milder alkalies preferably being used in high temperature digestions, as they are then more effective than at lower temperatures. When comparatively concentrated alkaline liquor is employed, the acid-sulphite-digested kraft pulp may be digested at comparatively low temperatures,—for instance, room temperature. Thus, the washed, acid-sulphite-digested pulp may be digested as a 6% suspension in an alkaline liquor having an alkali concentration of from 5% to 8%, calculated as NaOH, at a temperature of, say, from 20° to 50° C. The alkali may consist of caustic soda alone, but a mixture of caustic soda and sodium sulphide is preferable, owing to the milder action of sodium sulphide. Such a digestion requires only from about one to two hours to go to completion.

After alkaline digestion, the pulp may be washed free of alkaline liquor, the resulting spent alkaline liquor preferably being reused, at least in part, particularly when it has a high content of unspent alkali. The alkaline-digested pulp may be bleached to a pure white color with a consumption of only about 5% to 6% bleach, based on fiber, and finally washed.

The process of the present invention may likewise advantageously include a treatment of the initially liberated kraft pulp with one or more lignin-reactive reagents, such as chlorine water or bleach liquor, before the pulp is subjected to alkaline digestion, particularly when the pulp used as a raw material is of an under-cooked or refractory variety and has a higher lignous content than usual. Such a treatment may be effected upon the raw pulp, or after the pulp has been digested in an acid-sulphite liquor, and in such case the washing of the pulp after such treatment, and the final alkaline digestion, results in a removal of lignin reaction products and facilitates final bleaching to high whiteness without a physical or chemical degradation of the fiber. The chlorine water or bleach liquor apparently does not react appreciably upon the pentosans present in the pulp, but, as stated, reacts upon and removes

lignin and allied substance, or renders such substance soluble in an alkaline liquor. Specifically, the procedure may be to steep a raw pulp, such as kraft, for about two to three hours in chlorine water at room temperature, containing, say, 3% to 4% chlorine, based on the weight of dry fiber, and then, preferably after washing, to digest the pulp successively in an acid-sulphite liquor and in an alkaline liquor, and finally to bleach the pulp as hereinbefore described. If desired, in lieu of treating with chlorine water, the pulp may be steeped in bleach liquor containing, say, 2% to 3% bleach, based on the dry weight of fiber, under the conditions hereinbefore given for the chlorine water treatment. Or the pulp may be treated, as described, successively with chlorine water and bleach liquor, or vice versa. Or either or both these treatments may be carried out after acid sulphite digestion rather than before such digestion. When bleach liquor is employed, it may be maintained distinctly alkaline during the treatment, by the addition of an alkali such as caustic soda, to avoid formation of oxycelluloses.

While a kraft pulp which has been digested in an acid-sulphite liquor containing more free than combined  $\text{SO}_2$  may be improved to a greater extent by alkaline digestion than a pulp which has been digested in an acid-sulphite liquor containing no more free than combined  $\text{SO}_2$ , (as in such first instance the pulp suffers marked depreciation both physically and chemically), nevertheless, even in such second instance it is, in certain cases, advantageous to digest the sulphite-digested pulp in an alkaline liquor before bleaching, in order to refine the pulp to higher alpha cellulose content by the removal of reaction products of acid sulphite digestion and other non-alpha cellulose impurities. Consequently, while the present process may be more effectively practiced by a two-step treatment of kraft or soda pulp, in which the first or acid sulphite digestion is accomplished by a cooking liquor having the free  $\text{SO}_2$  content higher than the combined  $\text{SO}_2$  content, I do not confine myself thereto as the invention may be practiced by carrying on the acid sulphite digestion in a cooking liquor in which the combined  $\text{SO}_2$  is equal to or greater than the free  $\text{SO}_2$ .

While the specific examples hereinbefore given deal specifically with kraft pulp, the process of the present invention may also be applied to advantage when soda pulp or other pulp liberated by the action of an alkaline liquor is used as a raw material. It will further be evident to those skilled in the art that various other changes or modifications might be made in the process of the present invention without departing from the spirit or scope of the appended claims. By the expression "more free than combined  $\text{SO}_2$ ," I

mean  $\text{SO}_2$  in excess of that necessary to form the acid sulphite or bisulphite of metals such as calcium, magnesium, sodium, or the like.

I claim:

1. A process which comprises digesting cellulose pulp in an acid-sulphite liquor containing more free than combined  $\text{SO}_2$ , and then digesting the pulp in an alkaline liquor to remove the products of hydrolysis resulting from said first-mentioned digestion. 70

2. A process which comprises digesting wood pulp liberated by the action of an alkaline liquor in an acid-sulphite liquor containing more free than combined  $\text{SO}_2$  to remove ligneous matter, pentosans, and other impurities from such pulp, and then digesting the pulp in an alkaline liquor to remove the products of hydrolysis resulting from said first-mentioned digestion. 75 80

3. A process which comprises digesting wood pulp, liberated by the action of an alkaline liquor, in an acid-sulphite liquor containing more free than combined  $\text{SO}_2$  to remove ligneous matter, pentosans, and other impurities from such pulp, then digesting the pulp in an alkaline liquor to remove the products of hydrolysis resulting from said first-mentioned digestion, and bleaching the alkaline-digested pulp. 90

4. A process which comprises digesting kraft pulp in an acid-sulphite liquor containing more free than combined  $\text{SO}_2$  to remove ligneous matter, pentosans, and other impurities from such pulp, washing the pulp, digesting the washed pulp in an alkaline liquor to remove the products of hydrolysis resulting from said first-mentioned digestion, washing the alkaline-digested pulp, and bleaching. 95 100

5. A process which comprises digesting raw pulp, previously liberated from the raw cellulosic material, in an acid-sulphite liquor to remove non-alpha cellulose components including ligneous matter and pentosans, then digesting the pulp in an alkaline liquor to remove more non-alpha cellulose components, and finally bleaching. 105 110

6. A process which comprises digesting wood pulp, previously liberated by the action of an alkaline liquor, in an acid-sulphite liquor to remove non-alpha cellulose components including ligneous matter and pentosans, then digesting the pulp in an alkaline liquor to remove more non-alpha cellulose components, and finally bleaching. 115 120

7. A process which comprises steeping raw pulp in a lignin-reactive reagent, digesting the pulp in an acid-sulphite liquor, digesting the pulp in an alkaline liquor, and finally bleaching. 125

8. In a process which includes digesting wood pulp in an acid-sulphite liquor and then digesting the pulp in an alkaline liquor, that step before alkaline digestion which

comprises treating the pulp with a lignin-reactive reagent.

9. A process which comprises digesting wood pulp liberated by the action of alkaline liquor in an acid sulphite liquor, washing the pulp, digesting the washed pulp in an alkaline liquor, washing the alkaline-digested pulp, and finally bleaching in hypochlorite bleach liquor.

10. In testimony whereof I have affixed my signature.

GEORGE A. RICHTER.

15

20

25

30

35

40

45

50

55

60

65